

# UNITED STATES PATENT OFFICE.

ADOLF BAEYER, OF MUNICH, BAVARIA, AND HEINRICH CARO, OF MANNHEIM, BADEN, GERMANY, ASSIGNORS TO THE BADISCHE ANILIN AND SODA FABRIK, OF MANNHEIM, BADEN, GERMANY.

## DYEING FABRICS WITH ARTIFICIAL INDIGO-BLUE.

SPECIFICATION forming part of Letters Patent No. 240,360, dated April 19, 1881.

Application filed February 15, 1881. (Specimens.)

To all whom it may concern:

Be it known that we, ADOLF BAEYER, a subject of the King of Bavaria, and HEINRICH CARO, of Mannheim, a subject of the Grand 5 Duke of Baden, residing, respectively, at Munich, in the Kingdom of Bavaria, and at Mannheim, in the Grand Duchy of Baden, Empire of Germany, have invented new and useful Improvements in Developing Blue Colors Within 10 in and Upon Textile Fibers and Fabrics from Artificial Indigo-Blue, of which the following is a specification.

This invention is based on the discovery that blue colors can be produced from orthonitrophenylpropionic acid within and upon textile fibers, yarn, or cloth. The said blue colors belong to the class of so-called "artificial indigo" which is produced according to the specification in Letters Patent No. 227,470, dated May 20 11, 1880, by the action of alkalies and deoxidizing agents upon orthonitrophenylpropionic acid. The said blue color is capable of replacing vegetable indigo-blue or similar blues in some of their industrial applications.

Now, we have discovered that the deoxidation of orthonitrophenylpropionic acid may also be effected by the action of deoxidizing sulphur compounds belonging to the class of sulpho-carbonates, and we have found that more especially with the aid of alkaline xanthates 30 good results are obtained; and our invention consists in the formation of blue colors belonging to the class of "artificial indigo-blue" within and upon a textile fiber, yarn, or cloth by the 35 means described in this specification.

In carrying out this invention we proceed as follows:

For printing purposes we prepare a printing-color suitable for calico-printing by mixing about ten parts, by weight, of orthonitrophenylpropionic acid and about four parts, by weight, of carbonate of potash with about one hundred parts, by weight, of starch-paste or any other suitable thickening. We then add in the cold 40 about fifteen parts, by weight, of xanthate of soda and mix well. The color thus prepared is ready for use, and ought to be employed for printing without much delay, as upon standing the color is liable to decompose. The text-

ile fiber, yarn, or cloth may also be first prepared, printed, or impregnated with a solution of xanthate of soda, and then be printed with a solution of an alkaline salt of orthonitrophenylpropionic acid; or the textile fiber, yarn, or cloth may be first prepared, printed, or impregnated with the alkaline salt of orthonitrophenylpropionic acid, and then be printed with the xanthate of soda.

The above-described mixtures and solutions can also be used as marking-inks for marking 60 textile fibers and fabrics.

After printing or marking by any of the above-described methods the blue color becomes developed within or upon the fiber, yarn, or cloth by mere aging at a moderate temperature—say about 20° to 50° centigrade. Steaming or heating is not required. After the color is fully developed the printed goods are washed and finished in the usual manner.

For dyeing purposes we prepare a cold aqueous solution with about ten parts, by weight, of orthonitrophenylpropionic acid, about four parts, by weight, of carbonate of potash, and about fifteen parts, by weight, of xanthate of soda, and with this solution we impregnate 75 the materials to be dyed in the usual way. For dark shades a concentrated solution is to be employed, and for light shades the solution is to be diluted accordingly. We then allow the goods to age in the usual manner at a moderate temperature—say about 20° to 50° centigrade—until the blue color becomes developed within or upon the fiber, yarn, or cloth. Subsequently the goods are washed and finished 80 in the usual way.

Having employed the term "orthonitrophenylpropionic acid" in this specification, we wish it to be understood that we do not intend to designate thereby a chemically pure substance bearing that name in scientific language, 90 but we intend to designate therewith a manufactured commercial product.

What we claim as new, and desire to secure by Letters Patent, is—

1. The within-described process for developing blue colors or dyes belonging to the class of artificial indigo-blue in or upon a textile fiber, yarn, or cloth, whether knit or woven,

by impregnating said fiber, yarn, or cloth with a solution of a mixture of orthonitrophenylpropionic acid and alkali and a deoxidizing sulphur compound belonging to the class of sulpho-carbonates, such as xanthates of soda, and then submitting the fiber, yarn, or cloth to a drying or aging process, substantially as set forth.

2. As a new article of manufacture, textile fibers, yarn, or cloth, whether knit or woven,

having the herein-described blue color developed within and upon the same.

In testimony whereof we have hereunto set our hands in the presence of two subscribing witnesses.

ADOLF BAEYER.  
HEINRICH CARO.

Witnesses:

PAUL FRIEDLAENDER,  
WILHELM HAUSSMANN.